

## UNITED STATES PATENT OFFICE

2,334,245

## CUTTING TOOL

Charles O. Burgess and William D. Forgeng,  
Niagara Falls, N. Y., assignors to Haynes Stellite  
Company, a corporation of Indiana

No Drawing. Original application July 30, 1940,  
Serial No. 348,445, now Patent No. 2,297,687,  
dated October 6, 1942. Divided and this ap-  
plication November 15, 1941, Serial No. 419,287

2 Claims. (Cl. 29—95)

This invention relates to abrasion resistant al-  
loys of the type composed principally of chro-  
mium and iron, and to new and useful cutting  
tools made therefrom. This application is a division  
of our copending application, Serial No.  
348,445, filed July 30, 1940, which has matured  
into Patent No. 2,297,687, of October 6, 1942.

Chromium-iron alloys, often modified by the  
addition of other elements, have been used to  
resist wear and abrasion. By varying the com-  
position, and in some instances the heat treat-  
ment, it has been possible to vary the hardness,  
toughness, and strength of the alloys over wide  
ranges. But hardness of a very high degree such  
as is required of a metal-cutting tool has here-  
tofore been accompanied by an undue degree of  
brittleness. Cutting tool "high speed" steels have  
been basically tungsten-iron compositions rather  
than chromium-iron, and have typically con-  
tained 18% tungsten, 4% chromium, and 1%  
vanadium (so-called "18-4-1") sometimes modi-  
fied by the addition of one or more of the metals,  
cobalt, nickel, and molybdenum.

It is a primary object of the invention to pro-  
vide an abrasion resistant chromium iron alloy  
which, in the form of a cutting tool, will cut met-  
als at high speeds at least as well as 18-4-1 high  
speed steel.

We have discovered that a hard chromium-iron  
alloy containing between 45% and 65% chromium  
is considerably toughened by the addition of car-  
bon in a percentage between 1% and 3%. For  
some purposes the carbon content may be some-  
what above or below that range. We have further  
found that the general suitability of such an alloy  
for use as a cutting tool and other abrasion-  
resisting articles is enhanced by the addition of  
the elements cobalt, nickel, silicon and one or  
more of the following elements: tungsten; molyb-  
denum; columbium; tantalum; titanium; vanadi-  
um; and zirconium in certain proportions here-  
inafter described.

More specifically, according to the invention,  
chromium alloys and cutting tools comprise com-  
positions substantially within the following per-  
centage limits:

|                        | Broad     | Preferred   |
|------------------------|-----------|-------------|
| Per cent chromium..... | 45 to 65  | 50 to 56    |
| Per cent cobalt.....   | 5 to 20   | 7 to 15     |
| Per cent nickel.....   | 4 to 20   | 6 to 15     |
| Per cent silicon.....  | 0.05 to 5 | 0.2 to 2    |
| Per cent carbon.....   | 1 to 3    | 1.5 to 2.25 |

With one or more of the elements tungsten, 55

molybdenum, columbium, tantalum, titanium,  
vanadium, and zirconium, in individual percent-  
ages not exceeding 5% and in a total aggregate  
percentage, including the silicon percentage,  
under 10%, the remainder iron, the iron being  
maintained above 15%. On occasion it will be  
desirable to add manganese up to about 10%.  
The normal impurities of steels, such as phos-  
phorus, sulfur, and nitrogen, may be present in  
small fractional percentages without departing  
from the invention.

The alloy tools of this invention may be used  
in the as-cast condition (after casting in sand or  
carbon molds for instance) or when heat treated.  
A suitable heat treatment consists in holding the  
alloy tools at a temperature between about 550°  
C. and about 850° C. for a time between about  
five minutes at the higher temperatures to about  
twenty hours at the lower temperatures. The  
alloys are hot forgeable to a limited extent. If  
the alloys are to be forged, it is best to begin that  
operation before they have cooled from the cast-  
ing step to below 900° C. Some cold deformation  
of the forged alloy can be effected, preferably  
after quenching from above 900° C.

Depending chiefly upon the composition and  
heat treatment, the hardness of the alloy of the  
invention varies between the approximate limits of  
30 55 to 70 Rockwell "C." The best cutting tool  
quality is usually attained in tools having a hard-  
ness in the neighborhood of 60 Rockwell "C." The  
transverse strength of the as-cast alloy is  
upwards of 1000 pounds (loading applied centrally  
35 to a section 0.5 inch by 0.5 inch square, sup-  
ported in a 4 inch span) and in the preferred  
range of compositions attains 3000 to 4000 pounds  
and sometimes more.

40 Cutting tests indicate that the alloy tool of the  
invention compares favorably with standard high  
speed steel tools of the 18-4-1 type. In accelerated  
life tests, cutting steel billets and semi-steel  
billets, and using surface speeds, feeds, and cuts  
45 considerably greater than normal, tools of this  
invention cut from two to eight times as far  
as standard "Rex AAA," a widely used high speed  
steel of high quality.

Although the use of the alloy of this invention  
as a cutting tool has been emphasized in the  
50 foregoing description, the alloy is capable of many  
other uses which are within the invention, for  
instance as a hard-facing material for tool and  
machinery wear-resisting parts.

We claim:

1. A heat-treated, high speed, metal-cutting

tool having substantially the composition: between 50% and 65% chromium, between 5% and 20% cobalt, between 4% and 20% nickel, between 0.05% and 5% silicon, between 1.5% and 3% carbon, a substantial amount of at least one of the elements from the group consisting of tungsten, molybdenum, columbium, tantalum, titanium, vanadium, and zirconium, in individual percentages not exceeding 5% and in an aggregate percentage, including the silicon percentage, under 10%, remainder iron; and being in the condition resulting from being heated at a temperature within the range 550° C. to 850° C. for a time between five minutes and twenty hours.

2. A heat-treated, high speed, metal-cutting tool having substantially the composition: 50% to

56% chromium, 7% to 15% cobalt, 6% to 15% nickel, 0.2% to 2% silicon, 1.5% to 2.25% carbon, a substantial amount of at least one of the elements from the group consisting of tungsten, molybdenum, columbium, tantalum, titanium, vanadium and zirconium, in individual percentages not exceeding 5% and in an aggregate percentage, including the silicon percentage, under 10%, remainder iron, the iron content being more than 15%; and being in the condition resulting from being heated at a temperature within the range 550° C. to 850° C. for a time between five minutes and twenty hours.

CHARLES O. BURGESS.  
WILLIAM D. FORGENG.